

## 1

2,902,394

 PROTECTIVE METAL COATING COMPOSITIONS  
AND METHOD OF COATING

Bruno R. Jeremias, Detroit, Mich., assignor to Poor &amp; Company, Chicago, Ill., a corporation of Delaware

 No Drawing. Application July 19, 1956  
Serial No. 598,762

8 Claims. (Cl. 148—6.21)

This invention relates to protective metal finishing compositions and more particularly to a metal finishing composition which can be applied to zinc surfaced articles to provide improved appearance and enhanced corrosion protection.

One of the objects of the invention is to provide a new and improved corrosion protecting metal finishing composition which produces a beautiful bronze color on zinc surfaces, for example, die cast zinc articles.

Another object of the invention is to provide a composition of the type described which produces enhanced corrosion protection on zinc surfaces.

Another object of the invention is to provide a new and improved method of producing excellent bronze corrosion resistant finishes on zinc surfaced articles. Other objects will appear hereinafter.

In accordance with the invention new and improved metal finishing coating compositions are prepared by intimately mixing chromic acid, a reducing agent capable of reducing a minor proportion of the chromic acid to a state in which the chromium is present as trivalent chromium, acetic acid, sulfuric acid and nitric acid. This composition is initially prepared as a concentrate, preferably by mixing together chromic anhydride, sodium sulfite, acetic acid, sulfuric acid, nitric acid and water. The concentrate is then diluted in actual practice with a relatively large quantity of water so that the final bath which is employed as a finishing composition for metal surfaces only contains around 1.5% to 4% by volume of the original concentrate.

The best mode contemplated for the practice of the invention is illustrated by the following composition which constitutes the concentrate:

| Ingredients:                                      | Grams per liter |
|---------------------------------------------------|-----------------|
| Chromic anhydride (CrO <sub>3</sub> )             | 401.0           |
| Sodium sulfite (Na <sub>2</sub> SO <sub>3</sub> ) | 7.5             |
| Acetic acid                                       | 22.5            |
| Sulfuric acid                                     | 45.0            |
| Nitric acid                                       | 228.0           |

the remainder being water.

When this composition is diluted with water so that the resultant bath contains 1.5% to 4% by volume of the initial concentrate the said bath is an excellent corrosion protecting composition and provides a beautiful bronze finish on zinc surfaced articles. The general procedure in providing such a finish on such articles is to immerse the articles in the bath at ordinary temperatures (70° F. to 90° F.) for a period of 5 to 15 seconds, then rinse the article with water and dry.

In the practice of the invention the amount of chromium present in the concentrate preferably varies from a minimum of about 200 grams per liter to the saturation solubility in the concentrate at a temperature around 20° C.

In the previously described concentrate it is desirable that not more than 1/6 of the chromium initially present in the hexavalent state be reduced to the trivalent state.

## 2

Thus if sodium sulfite is used as the reducing agent the maximum amount of sodium sulfite in the concentrate previously described should not exceed about 50 grams per liter. The ratio of reducing agent to chromic acid in the concentrate should provide preferably at least 1 gram per liter and not more than 11 grams per liter of trivalent chromium.

The ratio of sulfuric acid to acetic acid is rather critical and should be approximately 2:1 on a weight basis. In the concentrate the minimum amount of acetic acid is about 20 grams per liter and the maximum amount of acetic acid preferably does not exceed about 40 grams per liter, the minimum amount of sulfuric acid is about 40 grams per liter and the maximum amount of sulfuric acid preferably does not exceed about 80 grams per liter.

The nitric acid serves to accelerate the action of the bath and in a concentrate of the type previously described preferably should not be less than 150 grams per liter nor more than 300 grams per liter.

In the final metal finishing bath prepared by dilution of the concentrate the amount of chromium should be within the range of 3 grams to 90 grams per liter, preferably 15 to 90 grams per liter. The ratio of SO<sub>4</sub><sup>2-</sup>:CrO<sub>4</sub><sup>2-</sup> should be within the range of about 1:4 to about 1:16 with optimum results being obtained at about 5.5:20. The treating bath made by diluting the concentrate in the manner previously described will contain about 0.3 gram per liter to about 0.6 gram per liter of acetic acid and about 0.6 gram per liter to about 1.2 grams per liter of sulfuric acid. The nitric acid in the treating bath will be about 2.25 grams per liter to about 4.5 grams per liter. The weight ratio of sulfuric acid to acetic acid in the metal finishing bath will be the same as the weight ratio in the concentrate, namely, approximately 2:1. The trivalent chromium in the treating bath should preferably be at least 0.015 gram per liter and not more than about 4.4 grams per liter.

Instead of the sodium sulfite other reducing agents can be used which are capable of reducing hexavalent chromium compounds to trivalent chromium compounds in acidic solutions, but it is desirable to employ reducing agents which do not form insoluble by-products with the acid of the acidic aqueous solution. Other examples of preferred reducing agents are sodium thiosulfate, sodium hydrosulfite, potassium sulfite, postassium thiosulfate, potassium hydrosulfite, ammonium sulfite, ammonium thiosulfate, and ammonium hydrosulfite. The hydrosulfites are also commonly referred to as hyposulfites. Other reducing agents which reduce chromic acid in acid solution can be used. Reducing agents such as calcium sulfite are undesirable because of the formation of insoluble calcium sulfate.

The reduction reaction between the chromate radical of the chromic acid and the sulfite radical which occurs when a sulfite such as sodium sulfite is mixed with the chromic acid in the presence of water can be expressed by the following equation:



The invention is especially useful in providing a beautiful bronze color and enhanced corrosion resistance to zinc die castings and to other zinc surfaced articles. An important advantage of the invention is that the metal to be treated can be immersed in the treating solution as previously described and requires no further treatment other than rinsing with water. In many types of chromic acid treatments heretofore proposed a secondary treatment is required. By the practice of the invention it is possible to produce zinc surfaced articles which show a high resistance to the formation of white corrosion products.

The expression "zinc surfaced article" is employed herein to cover any article having an exterior surface of zinc regardless of whether the article itself is made of zinc, a ferrous metal or some other metal capable of being coated with zinc. The expression "zinc plated article" is employed herein to describe a zinc coated article in which the zinc coating has been applied by an electroplating process.

The invention is hereby claimed as follows:

1. A process of finishing zinc surfaced articles which comprises treating the surfaces of such articles with an aqueous solution of chromic acid containing 3 to 90 grams per liter of chromium of which at least 0.015 gram per liter but not more than about 4.4 grams per liter is chromium in a trivalent state, the remainder being 15 chromium, in a hexavalent state, 0.3 to 0.6 gram per liter of acetic acid, 0.6 to 1.2 grams per liter of sulfuric acid, and about 2.25 grams per liter to 4.5 grams per liter of nitric acid, the weight ratio of sulfuric acid to acetic acid being approximately 2:1 and the weight ratio of  $\text{SO}_4^{2-}:\text{CrO}_4^{2-}$  being within the range of about 1:4 to 1:16.

2. A process as claimed in claim 1 in which the article to be treated is immersed in said aqueous solution at a temperature of 70° F. to 90° F. for a period of 5 to 15 seconds and then rinsed with water.

3. A process as claimed in claim 1 in which the ratio of  $\text{SO}_4^{2-}:\text{CrO}_4^{2-}$  is about 5.5:20.

4. An acidic aqueous metal treating solution consisting essentially of an aqueous solution of chromic acid containing about 3 to 90 grams per liter of chromium of which at least about 0.015 gram per liter but not more than about 4.4 grams per liter is chromium in a trivalent state, the remainder being chromium in a hexavalent state, 0.3 to 0.6 gram per liter of acetic acid 0.6 to 1.2 grams per liter of sulfuric acid and about 2.5 to 4.5 grams per liter of nitric acid, the weight ratio of sulfuric acid to acetic acid being approximately 2:1 and the weight ratio of  $\text{SO}_4^{2-}:\text{CrO}_4^{2-}$  being within the range of 1:4 to 1:16.

5. An acidic aqueous metal treating solution consisting essentially of an aqueous solution of chromic acid containing about 15 to 90 grams per liter of chromium of which at least about 0.015 gram per liter but not more than about 4.4 grams per liter is chromium in a trivalent state, the remainder being chromium in a hexavalent state 0.3 to 0.6 grams per liter of acetic acid, 0.6 to 1.2

grams per liter of sulfuric acid and about 2.5 to 4.5 grams per liter of nitric acid, the weight ratio of sulfuric acid to acetic acid being approximately 2:1 and the weight ratio of  $\text{SO}_4^{2-}:\text{CrO}_4^{2-}$  being within the range of 1:4 to 1:16.

6. A concentrate adapted to be added to water to produce an aqueous metal treating solution, said concentrate consisting essentially of an aqueous solution of chromic acid containing chromium in an amount from about 200 grams per liter to the saturation solubility in the solution at 20° C., of which at least 1 gram per liter and not more than 11 grams per liter is trivalent chromium, the remainder being chromium in a hexavalent state, 20 to 40 grams per liter of acetic acid, 40 to 80 grams per liter of sulfuric acid and 150 to 300 grams per liter of nitric acid, the weight ratio of sulfuric acid to acetic acid being approximately 2:1 and the weight ratio of  $\text{SO}_4^{2-}:\text{CrO}_4^{2-}$  being within the range of 1:4 to 1:16.

7. A concentrate as claimed in claim 6 in which sodium sulfite is present in an amount sufficient to produce trivalent chromium within the proportions stated.

8. An acidic aqueous metal treating concentrate adapted to be diluted with water to form a metal protecting material, said concentrate having the following approximate composition:

| Ingredients:                                | Grams per liter |
|---------------------------------------------|-----------------|
| Chromic anhydride ( $\text{CrO}_3$ )        | 401.0           |
| Sodium sulfite ( $\text{Na}_2\text{SO}_3$ ) | 7.5             |
| Acetic acid                                 | 22.5            |
| Sulfuric acid                               | 45.0            |
| Nitric acid                                 | 228.0           |

35 the remainder being water.

#### References Cited in the file of this patent

#### UNITED STATES PATENTS

|    |           |                |               |
|----|-----------|----------------|---------------|
| 40 | 2,035,380 | Wilhelm        | Mar. 24, 1936 |
|    | 2,628,925 | Ostrander      | Feb. 17, 1953 |
|    | 2,796,372 | Chester et al. | June 18, 1957 |

#### FOREIGN PATENTS

|    |         |               |               |
|----|---------|---------------|---------------|
| 45 | 586,517 | Great Britain | Mar. 21, 1947 |
|    | 489,887 | Great Britain | July 2, 1947  |
|    | 852,634 | Germany       | Oct. 16, 1952 |

UNITED STATES PATENT OFFICE  
CERTIFICATE OF CORRECTION

Patent No. 2,902,394

September 1, 1959

Bruno R. Jeremias

It is hereby certified that error appears in the printed specification of the above numbered patent requiring correction and that the said Letters Patent should read as corrected below.

Column 3, line 35, for "acetic acir" read -- acetic acid,--; line 47, after "state" insert a comma; column 4, line 46, list of references cited, under "FOREIGN PATENTS" for "489,887" read -- 589,887 --.

Signed and sealed this 23rd day of February 1960.

(SEAL)

Attest:

KARL H. AXLINE

Attesting Officer

ROBERT C. WATSON

Commissioner of Patents